

# UNITED STATES PATENT OFFICE.

CHARLES HASLWANTER, JR., OF NEW YORK, N. Y., ASSIGNOR TO  
HARWOOD HUNTINGTON, OF SAME PLACE.

## SAFETY-MATCH.

SPECIFICATION forming part of Letters Patent No. 664,609, dated December 25, 1900.

Application filed July 14, 1899. Serial No. 723,853. (No specimens.)

To all whom it may concern:

Be it known that I, CHARLES HASLWANTER, Jr., a citizen of the United States, and a resident of New York, (Brooklyn,) Kings county, State of New York, have invented new and useful Improvements in the Manufacture of Matches, of which the following is a specification.

This invention relates to improvements in headless safety-matches free from phosphorus and which are intended to ignite by striking against a suitably-prepared surface.

There have been for years attempts made to produce a non-hygrometric match which will not be injuriously affected by hygrometric changes in the atmosphere, and the match herewith brought forward possesses the desirable antihygroscopic properties to a high degree.

In my invention I use barium hydroxid with alkali or alkaline-earth chlorates. I impregnate several times, preferably in hot solutions, drying either partially or wholly between the impregnations. The barium hydroxid and the chlorate used must be sufficiently pure to avoid hygroscopicity by reason of impurities. When barium hydroxid and the chlorate of potassium are used, I have found that the following proportions work ad-

vantageously, although I do not limit myself to the proportions stated precisely: twenty-three (23) parts of chlorate of potassium, one and one-half ( $1\frac{1}{2}$ ) parts of barium hydroxid, and one hundred (100) parts of water. The

parts given are by weight. The solution is used hot, a temperature of about ninety degrees ( $90^\circ$ ) centigrade being employed. The splints or match ends may be dried previous to the first impregnation. After the splints

or match ends have been dipped in the mixture of chlorate and barium hydroxid the splints or match ends are dried either partially or wholly at a temperature preferably between forty-five ( $45^\circ$ ) and fifty-five degrees

( $55^\circ$ ) centigrade. The splints or match ends are then dipped again in the mixture of the chlorate and the barium hydroxid and dried again either wholly or partially. I find that it is advantageous to repeat this dipping or

impregnating several times, so that enough of the material is introduced into the points of the splints or match ends. Either or both ends of the splints or match ends may be dipped and impregnated. The splints or match ends may also be dipped in paraffin or similar substances, which act as flame-carriers or flame-continuers. The splints or match ends may now be covered with a varnish, so that the crystals on the exterior of the surface of the splints or match ends may not be rubbed off in the later processes of manufacture, boxing, and transportation. I am aware that gum-arabic has been used as a binding material. I am also aware that spirit or oil varnishes have been used to try to make the match waterproof, but not, as in my invention, to form a cover to protect from attrition or rubbing off. The varnish may be put on, preferably, by spraying, and I use a solvent which will not dissolve the chemicals already in the match end. I dissolve the rosin used in petroleum spirit one (1) part of rosin to four (4) parts of the solvent. The splints or match ends are lastly dried again and a temperature of about ninety ( $90^\circ$ ) degrees centigrade is desirable.

I do not limit myself to the proportions and temperatures given in the above examples; but I have found them to be advantageous and will enable any one skilled in the art to produce the match.

Having now described my invention and the manner in which the same can be performed and the product obtained thereby, what I claim, and desire to protect by Letters Patent, is—

A headless safety-match impregnated with barium hydroxid and chlorates substantially as described.

In testimony that I claim the foregoing as my invention I have signed my name, in the presence of two witnesses, this 27th day of March, 1900.

CHARLES HASLWANTER, JR.

Witnesses:

SIMEON B. CHITTENDEN,  
HARWOOD HUNTINGTON.